

1

3,666,476

THIO-SUBSTITUTED [2.2.1]BICYCLIC COMPOUNDS AS ANTIFOGGANTS FOR SILVER HALIDE EMULSIONS

John Robert Dann and William Frank Fowler, Jr., Rochester, N.Y., assignors to Eastman Kodak Company, Rochester, N.Y.  
No Drawing. Filed Nov. 28, 1969, Ser. No. 880,895  
Int. Cl. G03c 1/34

U.S. CL. 96—109

35 Claims

ABSTRACT OF THE DISCLOSURE

Photographic compositions containing thio-substituted polycyclic compounds. In one aspect, the thio-substituted compounds containing a thio-substituted [2.2.1] bicyclic moiety are good antifoggants in photographic silver halide compositions.

This invention relates to photographic compositions and in particular to photographic compositions containing certain thio-substituted polycyclic compounds. In one aspect, this invention relates to photographic compositions containing thio-substituted polycyclic compounds which provide improved antifoggant or stabilizing properties in said compositions. In another aspect, this invention relates to silver halide photographic compositions having a very useful combination of ingredients.

It is known that sulfur compounds such as mercaptans and simple thioethers can be used to sensitize silver halide emulsions, providing improved photographic speed such as, for example, in Dann and Chechak, U.S. Pat. 3,046,134 issued July 24, 1962. Various sulfur-containing and nitrogen-containing compounds have also been used as antifoggants in silver halide emulsions as disclosed in Glafkides, Photographic Chemistry, 1958, pp. 374-378. However, improved additives to silver halide compositions which provide increased stability, improved antifogging of the emulsion, improved speed and the like or combinations of these properties without adversely affecting others are desirable.

We have now found new photographic composition combinations which exhibit improved photographic properties and provide an improved image record. Generally, we have found that light-sensitive, photographic compositions used in combination with a thio-substituted polycyclic compound containing the moiety:



provide improved photographic properties, especially such improved properties as reduced fog and improved stability of the element. This improvement is quite unexpected since the thio substitution adjacent a [2.2.1] bridged ring would be expected to be quite inactive and inert.

One preferred embodiment of our invention relates to photographic compositions comprising compounds having a thio-substituted [2.2.1] bridged-ring moiety. Compounds containing this moiety can be macrocyclic compounds, but are preferably simple compounds containing at least one such moiety or polymeric compounds which contain recurring units wherein at least one of the recurring units contains this moiety.

In another preferred embodiment, the bridged ring is a divalent bridged Diels-Alder adduct of cyclopentadiene and a dieneophile.

Another preferred embodiment of this invention relates to photographic silver halide compositions comprising a thio substituted [2.2.1] bicyclic compound.

2

In another preferred embodiment, this invention relates to photographic compositions comprising a polymer which contains recurring units of the formula:



5 wherein D represents a polycyclic group containing a [2.2.1] bridged ring adjacent the thio atom. The polycyclic group can, of course, be substituted by various groups including additional cyclic groups, straight chain groups which preferably contain condensation groups such as esters, carbamides, urethanes and the like.

The thio-substituted compounds useful in the combinations of this invention can generally be made by reacting hydrogen sulfide, a monomercaptan or a bis-mercaptan with an unsaturated bridged-ring compound. Of course, intralinear groups in the case of polymers and macrocyclic compounds and external groups in the case of simple compounds, polymers and macrocyclic compounds can be present. A typical simple reaction involves the reaction of cycloalkadiene with a dienophile (i.e., having at least one double bond) by a reaction commonly known as a Diels-Alder reaction, such as those described in Organic Reactions, vol. IV, Chapters I and II, John Wiley and Sons, Inc., New York, 1948, to produce a bicyclo[2.2.1]-5-heptene. This Diels-Alder adduct is then reacted with the sulfur compound to provide a thio-substituted bicyclo[2.2.1] heptane.

Typical compounds useful in the photographic combinations of the invention contain a group generally represented by the formula:



35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 960

3

group where X is  $-\text{O}-$  or  $-\text{NH}-$ ; or  $\text{R}^1$  and  $\text{R}^4$  can additionally be a



group, and  $\text{R}^5$  is a hydrogen atom, an alkyl group including substituted alkyl groups and alkyl groups containing hetero atoms, i.e., oxygen, sulfur or nitrogen atoms, in or appended to the alkyl chain and alkyl groups terminated with an



group where  $m$ , A and  $\text{R}^1$  to  $\text{R}^4$  are as described above, for example, methyl, ethyl, propyl, butyl, carboxymethyl, 2,3 - dicarboxynorborn-5-ylthioethoxyethoxyethyl, acetyl, propionyl, butyryl, 1,2-dicarboxyethyl, carboxypropyl, ethoxycarbonylpropyl, methoxycarbonylethyl, 1,2 - bis (ethoxycarbonyl)ethyl, 2-(norborn-2-yl)ethylthioethyl, 2-(5,6 - dicarboxynorborn-2-yl)ethylthioethyl, hydroxypropyl, hydroxyethyl, hydroxymethyl, an aryl group such as phenyl or substituted phenyl; or the group



wherein  $m$ , A and  $\text{R}^1$  to  $\text{R}^4$  are as described above.

When the compounds of the invention are polymeric, they contain recurring units having structures represented by Formula I, II, III or IV as follows:

(I)



wherein  $m$ , A, and  $\text{R}^1$  and  $\text{R}^4$  individually, are as described above, and  $\text{R}^1$  and  $\text{R}^4$  together with the carbon atom to which they are attached can be a



group;  $\text{R}^6$  is an alkylene group including substituted, branched chain, and hetero atom-containing alkylene

75

4

groups, for example, ethylene, propylene, trimethylene, tetramethylene, ethyleneoxyethoxyethyl, hydroxymethyl-ethylene, ethylenethioethyl, and the like; G is selected from the group consisting of carboxymethylmethylen

5



carboxyethylene  
10  
and the group



15

wherein  $m$ , A, and  $\text{R}^1$  and  $\text{R}^4$  individually, are as described above; and  $\text{R}^7$  is an alkylene, cycloalkylene or arylene group, which is the condensation residue of a diol or a diamine, i.e., an  $-\text{O}-\text{R}^8-\text{O}-$ , an

20



an  $\text{NH}-\text{Ar}-\text{NH}$  or an



30

group wherein  $\text{R}^8$  is an alkylene, including substituted, branched chain and hetero atom-containing alkylene groups, including alkylene groups containing cycloalkylene groups therein, for example,  $\text{R}^7$  can be the groups:



and



45

and  $\text{Ar}$  is an aryl group;  $x$  is an integer of 1 or 2 provided that it is 1 when  $-\text{G}-$  is the group:



60

wherein  $\text{R}^1$  and  $\text{R}^4$  are taken together with the carbon atoms to which they are attached to be a

65



70

group;



wherein  $m$ , A, and  $R^1$  and  $R^4$  individually, and  $R^6$  are as described above,  $R^9$  is an alkylene group having 1 to 6 carbon atoms, preferably methylene; Y is an  $-\text{O}-$  or  $-\text{NH}-$  group and  $R^{10}$  is the condensation residue of an aliphatic or aromatic dicarboxylic acid, i.e., a



group wherein  $R''$  is an aromatic or aliphatic group such as phenylene, alkylene, phenylenebisalkylene, alkylenebis-phenylene, cycloalkylene, cycloalkylenebisalkylene, and the like, including alkylene groups containing hetero atoms and cycloalkylene groups therein, for example, the group:



III



wherein A, and  $R^1$  and  $R^4$  individually, are as described above and  $R^{12}$  is an alkylene group containing an ester



or amido



linkage, including substituted derivatives thereof, for example,



IV



wherein  $m$ , A, and  $R^1$  and  $R^4$  individually, are as described above and  $R^1$  and  $R^4$  taken together with the carbon atoms to which they are attached can be a

15



20 group;  $R^{13}$  is selected from any of the groups described for  $R^{12}$  and from groups having the structure:

25



30

wherein  $m$ , A,  $R^{12}$ , and  $R^1$  and  $R^4$  individually, are as described above, or when  $R^1$  and  $R^4$  are taken together with the atoms to which they are attached to form an

35



40

group,  $R^{13}$  is an alkylene, arylene, arylenebisalkylene or an alkylenebisarylene, for example, phenylenedimethylene, phenylene, methylenediphenylene, ethylene, tetramethylene, and the like.

45

The present invention and the above formulae are also intended to include the respective sulfoxide and sulfone compounds wherein the thio atom has been oxidized to a sulfoxide or a sulfone.

50

The polymeric compounds of this invention can be prepared by reacting sulfur compounds such as hydrogen sulfide or mono-and/or poly-functional mercaptans with a polycyclic compound containing an unsaturated [2.2.1] bicyclic moiety. Reaction conditions favoring free radical reactions are preferred. Reactions which proceed with difficulty are catalyzed by the use of free radical catalysts such as ascaridole, peroxides and the like, or ultraviolet

55

light, optionally with photosensitizers such as acetone, benzophenone, etc., and heat or combinations thereof. In general terms, the reaction proceeds by the addition of a mercaptan to the double bond of a [2.2.1] bicyclic moiety containing an unsaturated group. Additional functional groups such as condensable groups (i.e., alcohol, acid, amide, etc.) are generally present on the mercaptan or the polycyclic compound, especially if polymers or macrocyclic compounds are formed. The linear linkage can be completed by condensation reacting through these groups

60

or simultaneously with the mercaptan reaction with the double bond on the [2.2.1] bicyclic moiety.

65

The thio-substituted compounds of this invention are generally incorporated into the photographic composition by techniques generally known in the art and as described in U.S. Pat. 3,046,134. The concentration of the compounds is dependent on the particular improvement desired. In the instance of silver halide compositions, concentrations of about 0.010 mg. to about 10 g./mole of silver halide, and preferably about 0.5 mg. to about 1 g. per mole of silver halide, are desired.

The silver halide emulsions used with this invention can comprise silver chloride, silver bromide, silver bromo-iodide, silver chlorobromoiodide or mixtures thereof. The emulsions may be coarse or fine grain and can be prepared by any of the well-known procedures, e.g., single-jet emulsions, double-jet emulsions such as Lippmann emulsions, ammoniacal emulsions, or thiocyanate- or thioether-ripened emulsions such as those described in Nietz et al., U.S. Patent 2,222,264; Illingsworth, U.S. Patent 3,320,069; and McBride, U.S. Patent 3,271,157. Surface-image emulsions may be used or internal-image emulsions such as those described in Davey et al., U.S. Patent 2,592,250; Lowe et al., U.S. Patent 3,206,313; Berriman et al., U.S. Patent 3,367,778; and Bacon et al., Belgian Patent 704,255. If desired, mixtures of surface- and internal-image emulsions may be used as described in Luckey et al., U.S. Patent 2,996,382. Negative-type emulsions may be used or direct-positive emulsions such as those described in Leermakers, U.S. Patent 2,184,013; Kendall et al., U.S. Patent 2,541,472; Berriman, U.S. Patent 3,367,778; Schouivenaars, British Patent 723,019; Illingsworth, French Patent 1,520,821; Ives, U.S. Patent 2,563,785; Knott et al., U.S. Patent 2,456,953; and Land, U.S. Patent 2,861,885.

The emulsions used with this invention may be sensitized with chemical sensitizers, such as with reducing agents; sulfur, selenium or tellurium compounds; gold, platinum or palladium compounds; or combinations of these. Suitable procedure are described in Shepard, U.S. Patent 1,623,499; Allen, U.S. Patent 2,399,083; McVeigh, U.S. Patent 3,297,447; and Dunn, U.S. Patent 3,297,446.

The photographic elements of this invention may contain incorporated developing agents such as hydroquinones, catechols, aminophenols, 3-pyrazolidones, ascorbic acid and its derivatives, reductones and phenylenediamines. Combinations of developing agents can be employed in the practice of the invention. The developing agents can be in a silver halide emulsion and/or in another suitable location in the photographic element. The developing agents may be added from suitable solvents or in the form of dispersions as described in Yackel, U.S. Patent 2,592,368, and Dunn et al., French Patent 1,505,778.

The photographic and other hardenable layers used in the practice of this invention can be hardened by various organic or inorganic hardeners, alone or in combination, such as the aldehydes, and blocked aldehydes, ketones, carboxylic and carbonic acid derivatives, sulfonate esters, sulfonyl halides and vinyl sulfones, active halogen compounds, epoxy compounds, aziridines, active olefins, isocyanates, carbodiimides, mixed-function hardeners and polymeric hardeners such as oxidized polysaccharides such as dialdehyde starch and oxyguar gum and the like.

The photographic emulsions and elements described in the practice of this invention can contain various colloids alone or in combination as vehicles, binding agents and various layers. Suitable hydrophilic materials include both naturally occurring substances such as proteins, for example, gelatin, gelatin derivatives, cellulose derivatives; polysaccharides such as dextran, gum arabic and the like; and synthetic polymeric substances such as water-soluble polyvinyl compounds such as poly(vinylpyrrolidone), acrylamide polymers and the like.

The described photographic emulsion layers and other layers of a photographic element employed in the practice of this invention can also contain, alone or in combination with hydrophilic, water-permeable colloids, other synthetic polymeric compounds such as dispersed vinyl compounds such as in latex form and particularly those which increase the dimensional stability of the photographic materials. Suitable synthetic polymers include those described, for example, in U.S. Patents 3,142,568 of Nottorf issued July 28, 1964; 3,193,386 of White issued July 6, 1965; 3,062,674 of Houck, Smith and Yudelson issued Nov. 6, 1962; 3,220,844 of Houck, Smith and Yudelson

issued Nov. 30, 1965; 3,287,289 of Ream and Fowler issued Nov. 22, 1966; and Dykstra, U.S. Patent 3,411,911; particularly effective are those water-insoluble polymers of alkyl acrylates and methacrylates, acrylic acid, sulfo-alkyl acrylates or methacrylates, those which have cross-linking sites which facilitate hardening or curing and those having recurring sulfobetaine units as described in Canadian Patent 774,054.

The photographic layers and other layers of a photographic element employed and described herein can be coated on a wide variety of supports. Typical supports include cellulose nitrate film, cellulose ester film, poly(vinyl acetal) film, polystyrene film, poly(ethylene terephthalate) film, polycarbonate film and related films or resinous materials, as well as glass, paper, metal and the like. Typically, a flexible support is employed, especially a paper support, which can be partially acetylated or coated with baryta and/or an alpha-olefin polymer, particularly a polymer of an alpha-olefin containing 2 to 10 carbon atoms such as polyethylene, polypropylene, ethylenebutene copolymers and the like.

The photographic layers employed in the practice of this invention can contain plasticizers and lubricants such as polyalcohols, e.g., glycerin and diols of the type described in Milton, U.S. Patent 2,960,404; fatty acids or esters such as those described in U.S. Patent 2,588,765 and Duane, U.S. Patent 3,121,060; and silicone resins such as those described in Du Pont, British Patent 955,061.

The photographic layers employed in the practice of this invention may contain surfactants such as saponin, anionic compounds such as the alkyl aryl sulfonates described in Baldsiefen, U.S. Patent 2,600,831, and amphoteric compounds such as those described in Ben-Ezra, U.S. Patent 3,133,816.

The light-sensitive silver halide emulsion of the multi-layer photographic elements of the invention can conveniently be ortho-sensitized or pan-sensitized with spectral sensitizing dyes. For instance, these emulsions can be spectrally sensitized by treating with a solution of a sensitizing dye in an organic solvent or the dye may be added in the form of a dispersion as described in Owens et al., French Pat. 1,482,774. Sensitizing dyes useful in sensitizing such emulsions are described, for example, in U.S. Pats. 2,526,632 of Brooker and White issued Oct. 24, 1950; 2,503,776 of Sprague issued Apr. 11, 1950; 2,493,748 of Brooker et al.; and 3,384,486 of Taber et al. Spectral sensitizers which can be used include the cyanines, merocyanines, complex (trinuclear) cyanines, complex (trinuclear) merocyanines, styryls and hemicyanines. The cyanines may contain such basic nuclei as thiazoles, oxazoles, selenazoles or imidazoles. Such nuclei may contain sulfoalkyl, carboxyalkyl and alkylamino groups and may be fused to benzene or naphthalene rings either unsubstituted or substituted with halogen, phenyl, alkyl or alkoxy groups. The dyes may be symmetrical or unsymmetrical and may contain alkyl, phenyl or heterocyclic substituents on the polymethylene chain. The merocyanine dyes may contain the basic nuclei mentioned above as well as acid nuclei such as thiohydantoins, rhodanines, oxazolidenediones and barbituric acids. The acid nuclei may be substituted with alkyl groups, phenyl groups, carboxy groups, sulfo groups or amino groups. The emulsions may contain supersensitizing dye combinations such as those described in U.S. Pats. 2,739,964 by Brooker et al.; 2,688,545 by Carroll et al.; 2,701,198 by Carroll et al.; 2,739,149 by VanLare; and British Pat. 1,128,840 by Fuji; or the dyes may be supersensitized with ascorbic acid derivatives, azaindenes, cadmium salts, and organic sulfonic acids as described in U.S. Pats. 2,933,390 by McFall et al. and 2,937,089 by Jones et al.

The photographic layers used in the practice of this invention may be coated by various coating procedures including dip coating, air knife coating, curtain coating or extrusion coating using hoppers of the type described in

Beguin, U.S. Pat. 2,681,294. If desired, two or more layers may be coated simultaneously by the procedures described in Russell, U.S. Pat. 2,761,791, and Wynn, British Pat. 837,095.

This invention may be used with elements designed for colloid transfer processes such as described in Yackel et al., U.S. Pat. 2,716,059; silver salt diffusion transfer processes such as described in U.S. Pats. 2,352,014 by Rott, 2,543,181 by Land, 3,020,155 by Yackel and 2,861,885 by Land; color-image transfer processes such as described in U.S. Pats. 3,087,817, 3,185,567 and 2,983,606 by Rogers, 3,253,915 by Weyerts, 3,227,550, 3,227,551 and 3,227,552 by Whitmore et al., and 3,415,644, 3,415,645 and 3,415,646 by Land; and imbibition transfer processes as described in U.S. Pat. 2,882,156 by Minsk.

This invention may be used with elements designed for color photography, for example, elements containing color-forming couplers such as those described in U.S. Pats. 2,376,679 by Frohlich et al.; 2,322,027 by Vittum et al.; 2,801,171 by Fierke et al.; 2,698,794 by Godowsky; 3,227,554 by Barr et al.; and 3,046,129 by Graham; or elements to be developed in solutions containing color-forming couplers such as those described in U.S. Pats. 2,252,718 by Mannes and Godowsky; 2,592,243 by Carroll et al.; and 2,950,970 by Schwan.

Typical compounds useful in the practice of the invention are listed below or, in the instance of polymeric or macrocyclic compounds, they contain units as represented below wherein  $n$  is a positive integer.



| Sample number | Structure |
|---------------|-----------|
| 4.....        |           |
| 5.....        |           |
| 6.....        |           |
| 7.....        |           |
| 8.....        |           |
| 9.....        |           |
| 10.....       |           |
| 11.....       |           |
| 12.....       |           |
| 13.....       |           |
| 14.....       |           |

TABLE—Continued

| Sample number | Structure |
|---------------|-----------|
| 15.....       |           |
| 16.....       |           |
| 17.....       |           |
| 18.....       |           |
| 19.....       |           |
| 20.....       |           |
| 21.....       |           |
| 22.....       |           |
| 23.....       |           |
| 24.....       |           |
| 25.....       |           |
| 26.....       |           |

TABLE—Continued

| Sample number | Structure                                                                           |
|---------------|-------------------------------------------------------------------------------------|
| 27.....       |    |
| 28.....       |    |
| 29.....       |    |
| 30.....       |    |
| 31.....       |    |
| 32.....       |   |
| 33.....       |  |
| 34.....       |  |
| 35.....       |  |
| 36.....       |  |
| 37.....       |  |
| 38.....       |  |
| 39.....       |  |

TABLE—Continued

| Sample number | Structure |
|---------------|-----------|
| 40.....       |           |
| 41.....       |           |
| 42.....       |           |
| 43.....       |           |
| 44.....       |           |
| 45.....       |           |
| 46.....       |           |
| 47.....       |           |
| 48.....       |           |
| 49.....       |           |
| 50.....       |           |
| 51.....       |           |

TABLE—Continued

| Sample number | Structure |
|---------------|-----------|
| 52.....       |           |
| 53.....       |           |
| 54.....       |           |
| 55.....       |           |
| 56.....       |           |
| 57.....       |           |

This invention is further illustrated by the following examples. Additional examples of preparation of compounds of this type are disclosed in copending application U.S. Ser. No. 880,896, filed on even date herewith.

#### PREPARATION OF COMPOUNDS

Example 1.—Sample 9: Copoly[bicyclo[2.2.1] - 5 - heptene - 2,3 - dicarboxylic anhydride-bis(2-mercaptopoethyl)-sulfide-hexamethylene diamine]

Bicyclo[2.2.1]-5-heptene - 2,3-dicarboxylic anhydride, 50 32.8 grams (0.2 mole), is dissolved in 100 ml. of benzene and mixed with 15.4 grams (0.1 mole) of bis(2-mercaptopoethyl)sulfide. After 2 days, 1/2 of the benzene solution is stirred with an aqueous solution of 5.8 grams (0.05 mole) of distilled hexamethylene diamine and 0.1 mole of sodium hydroxide in 50 ml. of water. The mixture is heated to 80° C., left standing overnight at room temperature, mixed with ethyl acetate and extracted with water. The aqueous layer is acidified with dilute hydrochloric acid to give a white stringy polymer which is purified by three more precipitations from aqueous solutions of its sodium salt with acid followed by washing with water after each precipitation.

Analysis.—Calculated for  $C_{28}H_{36}N_2O_6S_3$  (percent): C, 56.7; H, 6.1; N, 4.7; S, 16.2; [N.E.], 296. Found (percent): C, 53.0; H, 7.2; N, 4.1; S, 15.3; [N.E.], 284.

Example 2.—Sample 14: Copoly[1,2 - bis(2 - mercaptoethoxy)ethane-dodecahydro - 1,4:5,8 - dimethanoanthraquinonylene-2,6 (or 7)]

1,4,4a,5,8,8a,9a,10a - octahydro - 1,4:5,8 - dimethano-9,10-anthraquinone, 12 grams (0.05 mole), and 1,2-bis (2-mercaptopoethoxy)ethane, 9.1 grams (0.05 mole), are mixed with 4 drops of ascaridole, the temperature rising spontaneously from 24° C. to 32° C. in 2 minutes. The re-

action mixture is then heated for 24 hours and precipitated from benzene with methanol.

Analysis.—Calculated (percent): C, 62.5; H, 7.1; S, 15.1. Found (percent): C, 61.0; H, 7.1; S, 14.9; MW, 460.

Example 3.—Sample 19: 5-carboxymethylmercaptopo-bicyclo[2.2.1]heptene-2,3-dicarboximide

Bicyclo[2.2.1] - 5 - heptene - 2,3 - dicarboximide, 8.7 grams (0.053 mole), and 19.5 grams (0.21 mole) mercaptoacetic acid are mixed with 4 drops of ascaridole and heated for 1 hour on the steam bath. Two more drops of ascaridole are added and the heating is continued for an additional 10 hours. The crystals which form are washed with benzene and recrystallized from ethyl acetate. Melting point: 151°-152° C.

Analysis.—Calculated for  $C_{11}H_{13}NO_4S$  (percent): C, 51.7; H, 5.10; N, 5.50; S, 12.5. Found (percent): C, 51.3; H, 5.3; N, 5.3; S, 12.2.

Example 4.—Sample 38

5,5' (or 5,6') - thiobis[bicyclo[2.2.1]heptane - 2,3-dicarboxylic acid anhydride], 9.62 grams (0.0265 mole), is dissolved in 500 ml. of glacial acetic acid and 6 ml. of 32 percent aqueous hydrogen peroxide is added. The reaction mixture is allowed to stand for 48 hours at room temperature. The solution is heated for 1 hour on a steam bath, the solvent is removed and the residue is taken up in hot ethyl acetate. Benzene is added to produce a cloud point and, after standing for several weeks, 10 grams of white crystals separate. Melting point >310° C. Analysis indicates that the product is the tetrabasic acid. After drying overnight under vacuum at 185° C., the anhydride is formed in quantitative yield.

## Example 5.—Sample 41

Equimolar amounts of mercaptosuccinic acid and bicyclo[2.2.1]-2-methyl - 3,3-dihydroxymethyl-5-heptene are mixed at room temperature in an inert atmosphere of nitrogen. After the initial exothermic reaction subsides, a small quantity (2-4 drops) of ascaridole is added. The reaction mixture is heated for several hours at  $\approx 1$  mm. Hg in the presence of an esterification catalyst. Upon completion of the reaction and cooling to room temperature, a hard, glassy solid forms.

*Analysis.*—Calculated for  $C_{14}H_{20}SO_5$  (percent): C, 56.0; H, 6.67; S, 10.65. Found (percent): C, 55.2; H, 6.7; S, 10.7.

## Example 6.—Sample 45

A mixture of 3 - methylbicyclo[2.2.1]-5-heptene-2-yl-methyl 3 - methylbicyclo[2.2.1]-5-heptene-2-carboxylate, 68 grams (0.25 mole), and benzophenone, 0.375 gram (0.00206 mole), are dissolved in 375 ml. of cyclohexane in a 500-ml. quartz flask equipped with a magnetic stirrer, a sintered glass bubbling tube and an outlet tube. The reaction mixture is stirred while hydrogen sulfide gas is bubbled into the solution. The flask is irradiated with a 275-watt sun lamp placed 1 inch from the outer surface of the flask. After 70 hours of reaction, the hot solution ( $68^\circ$  C.) is allowed to cool to room temperature and an insoluble oil settles out.

The oil is dissolved in 100 ml. of ethyl acetate, precipitated in 700 ml. of ethyl alcohol, dissolved in 200 ml. of methylene chloride and precipitated twice in 600 ml. of acetone. The product is then dried in a vacuum oven at  $117^\circ$  C. for 1 hour to yield 50 grams (65% yield) of a brittle, glassy polymer.

## Example 7.—Sample 51

A mixture of 4,4' - methylenedianiline, 4.955 grams (0.025 mole), and dry dimethyl acetamide, 94 ml. (distilled from phosphorus pentoxide), is placed in a flamed 250-ml. flask equipped with a nitrogen tube, magnetic stirrer and drying tube. 5,5' (or 5,6') - thiobis(bicyclo[2.2.1]heptene-2,3 - dicarboxylic acid anhydride), 9.06 grams (0.025 mole), is added with stirring to the above mixture. The reaction mixture is stirred under nitrogen for 17 hours and then stored in a freezer.

The reaction mixture is placed on a glass plate, heated under nitrogen for 20 minutes at  $80^\circ$  C., held at 400 microns of Hg for 1 hour at  $25^\circ$  C. and then held under nitrogen for 1 hour at  $300^\circ$  C. The resulting polymer is a clear, hard resin.

The same compound can be prepared by reacting the half-ester (dimethyl) of the bisanhydride above with 4,4'-methylenedianiline.

## Example 8.—Sample 56

5,5' ( or 5,6' ) - thiobis(bicyclo[2.2.1]heptane- 2,3-dicarboxylic acid anhydride) is hydrolyzed with 4 parts of sodium hydroxide in water and then acidified with dilute hydrochloric acid. The product is the tetrabasic acid shown above.

## Example 9

Samples of the compounds listed above are added to a coarse-grained silver bromoiodide emulsion which contains 6.25 mole percent iodide and which is panchromatically sensitized with a cyanine dye. The emulsion samples are coated on a cellulose acetate support at a coverage of 459 mg. of silver and 1040 mg. of gelatin per square foot. Samples of the coatings are exposed on an Eastman 1B sensitometer, processed for 5 minutes in Kodak Developer DK-50, fixed, washed and dried.

Results of tests run on sample coatings are set forth in Table 1.

TABLE 1

| 5       | Sample No. | Concen- tration, g./mole | Fresh test |          |      | Incubation at 120° F., 50% RH |          |     | No. of week |  |
|---------|------------|--------------------------|------------|----------|------|-------------------------------|----------|-----|-------------|--|
|         |            |                          | Ag speed   | $\gamma$ | Fog  | Relative speed                | $\gamma$ | Fog |             |  |
|         |            |                          |            |          |      |                               |          |     |             |  |
| 1       | 0.9        | 110                      | 1.22       | 0.16     | 89   | 1.05                          | 0.16     | 2   |             |  |
| Control |            | 100                      | 1.25       | 0.15     | 44   | 0.75                          | 0.72     | 2   |             |  |
| 2       | 0.75       | 67                       | 1.07       | 0.10     | 65   | 0.92                          | 0.12     | 2   |             |  |
| 3       | 0.75       | 68                       | 1.05       | 0.13     | 29.5 | 0.90                          | 0.15     | 2   |             |  |
| 4       | 0.75       | 59                       | 1.05       | 0.11     | 23   | 0.92                          | 0.15     | 2   |             |  |
| Control |            | 100                      | 1.23       | 0.10     | 33   | 0.57                          | 0.87     | 2   |             |  |
| 5       | 0.15       | 94                       | 1.25       | 11       | 71   | 1.13                          | .15      | 2   |             |  |
| Control |            | 100                      | 1.28       | .14      | 10.2 | .53                           | 1.29     | 2   |             |  |
| 6       | 0.3        | 89                       | 1.30       | .11      | 69   | 1.07                          | .12      | 2   |             |  |
| Control |            | 100                      | 1.47       | .11      | 20   | .67                           | .97      | 2   |             |  |
| 7       | 0.9        | 87                       | 1.43       | .17      | 48   | .87                           | .14      | 2   |             |  |
| Control |            | 100                      | 1.58       | .16      | 12.3 | .70                           | .77      | 2   |             |  |
| 8       | 0.3        | 97                       | 1.13       | .10      | 83   | 1.02                          | .20      | 2   |             |  |
| Control |            | 100                      | 1.17       | .12      | 7.3  | .45                           | 1.28     | 2   |             |  |
| 9       | 0.3        | 76                       | 1.32       | .15      | 63   | 1.07                          | .11      | 2   |             |  |
| Control |            | 100                      | 1.55       | .17      | 12.6 | .60                           | 1.15     | 2   |             |  |
| 10      | 0.15       | 91                       | 1.27       | .10      | 74   | 1.07                          | .14      | 2   |             |  |
| Control |            | 100                      | 1.18       | .12      | 14   | .62                           | 1.11     | 2   |             |  |
| 11      | 0.3        | 80                       | 1.23       | .10      | 46   | .87                           | .20      | 2   |             |  |
| Control |            | 100                      | 1.42       | .11      | 12.6 | .62                           | 1.01     | 2   |             |  |
| 12      | 0.3        | 107                      | 1.17       | .11      | 65   | .98                           | .34      | 2   |             |  |
| Control |            | 100                      | 1.17       | .12      | 7.3  | .45                           | 1.28     | 2   |             |  |
| 13      | 7.2        | 82                       | .58        | .17      | 18   | .63                           | .10      | 2   |             |  |
| Control |            | 100                      | 1.25       | .10      | 13   | .58                           | .99      | 2   |             |  |
| 13      | 0.3        | 74                       | 1.12       | .11      | 63   | .90                           | .10      | 2   |             |  |
| Control |            | 100                      | 1.24       | .10      | 46   | .61                           | .82      | 2   |             |  |
| 14      | 0.6        | 87                       | 1.13       | .10      | 74   | 1.03                          | .14      | 2   |             |  |
| Control |            | 100                      | 1.02       | .14      | 22   | .52                           | 1.12     | 2   |             |  |
| 15      | 1.5        | 83                       | 1.42       | .08      | 42   | .98                           | .35      | 2   |             |  |
| Control |            | 100                      | 1.42       | .11      | 12.6 | .62                           | 1.01     | 2   |             |  |
| 16      | .60        | 58                       | 1.27       | .07      | 63   | .95                           | .18      | 2   |             |  |
| Control |            | 100                      | 1.18       | .10      | 32   | .62                           | .69      | 2   |             |  |
| 17      | .60        | 89                       | 1.47       | .14      | 67   | 1.10                          | .29      | 1   |             |  |
| Control |            | 100                      | 1.39       | .15      | 50   | .96                           | .65      | 1   |             |  |
| 18      | .60        | 97                       | 1.28       | .13      | 57   | .83                           | .56      | 2   |             |  |
| Control |            | 100                      | 1.28       | .15      | 49   | .67                           | .90      | 2   |             |  |
| 19      | 2.40       | 16                       | 1.35       | .07      | 29   | 1.23                          | .08      | 1   |             |  |
| Control |            | 100                      | 1.23       | .13      | 83   | .98                           | .49      | 1   |             |  |
| 20      | .90        | 73                       | 1.35       | .12      | 57   | .93                           | .23      | 2   |             |  |
| Control |            | 100                      | 1.36       | .15      | 32   | .65                           | .96      | 2   |             |  |
| 21      | .90        | 80                       | 1.18       | .12      | 62   | 1.07                          | .36      | 1   |             |  |
| Control |            | 100                      | 1.24       | .13      | 54   | .95                           | .53      | 1   |             |  |
| 22      | 3.00       | 80                       | 1.12       | .08      | 52   | 1.02                          | .26      | 2   |             |  |
| Control |            | 100                      | 1.28       | .12      | 17.5 | .68                           | 1.08     | 2   |             |  |
| 23      | .03        | 69                       | .93        | .13      | 59   | .80                           | .20      | 1   |             |  |
| 25      | .03        | 76                       | 1.08       | .11      | 63   | 1.07                          | .26      | 1   |             |  |
| 26      | .03        | 63                       | 1.17       | .10      | 53   | .98                           | .24      | 1   |             |  |
| 28      | .006       | 69                       | 1.12       | .10      | 59   | .98                           | .27      | 1   |             |  |
| 29      | .03        | 97                       | 1.15       | .11      | 91   | 1.02                          | .20      | 1   |             |  |
| 30      | .03        | 97                       | 1.08       | .13      | 83   | 1.00                          | .26      | 1   |             |  |
| Control |            | 100                      | 1.15       | .13      | 74   | .90                           | .44      | 1   |             |  |
| 24      | .30        | 67                       | 1.10       | .09      | 39   | .87                           | .45      | 2   |             |  |
| 27      | .03        | 87                       | 1.07       | .15      | 71   | .93                           | .26      | 2   |             |  |
| 31      | .15        | 59                       | .90        | .12      | 55   | .65                           | .35      | 2   |             |  |
| Control |            | 100                      | 1.14       | .13      | 21.5 | .53                           | 1.09     | 2   |             |  |
| 32      | .30        | 85                       | 1.48       | .09      | 36   | .97                           | .41      | 2   |             |  |
| Control |            | 100                      | 1.40       | .10      | 12.3 | .61                           | .99      | 2   |             |  |
| 33      | 0.9        | 71                       | 0.98       | .07      | .71  | 0.85                          | .11      | 2   |             |  |
| Control |            | 100                      | 1.16       | .10      | 76   | 0.91                          | .20      | 2   |             |  |
| 34      | 0.9        | 89                       | 1.47       | .14      | 71   | 1.23                          | .20      | 2   |             |  |
| Control |            | 100                      | 1.68       | .18      | .29  | 0.86                          | 1.02     | 2   |             |  |
| 35      | 0.75       | 83                       | 1.47       | .11      | 47   | 1.13                          | .26      | 2   |             |  |
| 36      | 0.75       | 85                       | 1.13       | .12      | 50   | 1.13                          | .31      | 2   |             |  |
| 37      | 0.75       | 100                      | 1.48       | .12      | 60   | 1.05                          | .28      | 2   |             |  |
| Control |            | 100                      | 1.28       | .15      | 41   | 1.05                          | .59      | 2   |             |  |
| 39      | 0.06       | 82                       | 1.32       | .19      | 82   | 1.27                          | .22      | 2   |             |  |
| Control |            | 100                      | 1.32       | .16      | 38   | .82                           | .85      | 2   |             |  |
| 40      | 0.6        | 69                       | 1.23       | .13      | 57   | 1.05                          | .13      | 2   |             |  |
| Control |            | 100                      | 1.25       | .10      | 63   | 1.01                          | .28      | 2   |             |  |
| 41      | 0.3        | 87                       | 1.55       | .14      | 58   | 1.18                          | .22      | 2   |             |  |
| 42      | 0.9        | 78                       | 1.52       | .17      | 57   | 1.30                          | .34      | 2   |             |  |
| 43      | 0.3        | 65                       | 1.47       | .17      | 52   | 1.22                          | .27      | 2   |             |  |
| Control |            | 100                      | 1.68       | .18      | 29   | .86                           | 1.02     | 2   |             |  |
| 44      | 0.75       | 82                       | 1.22       | .10      | 38   | 1.05                          | .49      | 2   |             |  |
| 45      | 0.75       | 100                      | 1.48       | .12      | 60   | 1.05                          | .28      | 2   |             |  |
| 46      | 0.75       | 74                       | 1.15       | .11      | 55   | 1.03                          | .27      | 2   |             |  |
| 47      | 0.15       | 80                       | 1.22       | .12      | 39   | 1.20                          | .40      | 2   |             |  |
| 48      | 0.75       | 89                       | 1.22       | .12      | 49   | 1.12                          | .35      | 2   |             |  |
| 52      | 0.75       | 94                       | 1.47       | .13      | 50   | 1.15                          | .40      | 2   |             |  |
| Control |            | 100                      | 1.28       | .15      | 41   | 1.05                          | .59      | 2   |             |  |
| 49      | 0.15       | 91                       | 1.27       | .12      | 55   | 1.07                          | .34      | 2   |             |  |
| 50      | 0.15       | 85                       | 1.28       | .18      | 57   | 1.02                          | .36      | 2   |             |  |
| 51      | 0.75       | 89                       | 1.30       | .12      | 62   | 1.05                          | .28      | 2   |             |  |
| Control |            | 100                      | 1.41       | .16      | 55   | .93                           | .50      | 2   |             |  |
| 53      | 2.4        | 76                       | 1.37       | .09      | 67   | 1.18                          | .13      | 2   |             |  |
| Control |            | 100                      | 1.48       | .13      | 60   | 1.13                          | .43      | 2   |             |  |
| 54      | 0.75       | 83                       | 1.35       | .11      | 50   | 1.08                          | .30      | 2   |             |  |
| 38      | 1.5        | 85                       | 1.27       | .12      | 58   | 1.00                          | .25      | 2   |             |  |
| Control |            | 100                      | 1.41       | .16      | 55   | .93                           | .50      | 2   |             |  |
| 55      | 1.5        | 91                       | 1.38       | .11      | 52   | 1.10                          | .40      | 2   |             |  |
| 56      | 1.5        | 82                       | 1.25       | .11      | 63   | 1.07                          | .27      | 2   |             |  |
| 57      | 0.15       | 85                       | 1.32       | .13      | 67   | 1.07                          | .31      | 2   |             |  |
| Control |            | 100                      | 1.47       | .16      | 44   | .99                           | .64      | 2   |             |  |

## Example 10

Some of the coatings of Example 9 containing the compounds listed above are given "forced development," i.e., development for 12 minutes in Kodak Developer DK-50, which is a longer development than is usually given, in

order to elicit any fogging tendencies of the compound. Sensitometric results given in Table 2 below show substantial lowering of fog in coatings containing the compounds of the invention.

TABLE 2

| Sample No. | Concen-<br>tration,<br>g./mole | Forced development |                        |          |
|------------|--------------------------------|--------------------|------------------------|----------|
|            |                                | Ag                 | Rel-<br>ative<br>speed | $\gamma$ |
| 16         | 0.6                            | 63                 | 1.30                   | .12      |
| Control    |                                | 100                | 1.21                   | .16      |
| 17         | 9.0                            | 67                 | 1.35                   | .16      |
| Control    |                                | 100                | 1.29                   | .23      |
| 22         | 3.0                            | 83                 | 1.42                   | .12      |
| Control    |                                | 100                | 1.28                   | .21      |
| 24         | 0.3                            | 83                 | 1.33                   | .14      |
| 26         | 0.03                           | 83                 | 1.23                   | .14      |
| 28         | 0.006                          | 83                 | 1.23                   | .16      |
| Control    |                                | 100                | 1.23                   | .24      |
| 39         | 1.5                            | 69                 | 1.72                   | .14      |
| Control    |                                | 100                | 1.43                   | .28      |
| 34         | 0.9                            | 85                 | 1.72                   | .19      |
| 42         | 0.9                            | 82                 | 1.57                   | .23      |
| 43         | 0.3                            | 78                 | 1.67                   | .22      |
| Control    |                                | 100                | 1.88                   | .30      |
| 55         | 7.2                            | 67                 | 1.42                   | .14      |
| Control    |                                | 100                | 1.75                   | .24      |
| 38         | 1.5                            | 83                 | 1.33                   | .20      |
| 54         | 0.75                           | 83                 | 1.50                   | .20      |
| Control    |                                | 100                | 1.38                   | .26      |

Although the invention has been described in considerable detail with particular reference to certain preferred embodiments thereof, variations and modifications can be effected within the spirit and scope of the invention.

We claim:

1. A silver halide photographic composition containing an antifogging concentration therein of (1) a simple compound having the structure:



wherein A is a methylene group, an oxygen atom, a sulfur atom or a >NH group; m is an integer of 1 to 4; R<sup>1</sup>, R<sup>2</sup>, R<sup>3</sup> and R<sup>4</sup> when taken separately are each a hydrogen atom, an alkyl, carboxy, mercapto, cyano, acylthio, or an alkanol group, or R<sup>1</sup>, R<sup>2</sup>, R<sup>3</sup> and R<sup>4</sup> taken together with the carbon atoms to which they are attached form a cyclopentene ring, a cyclopentane ring, a



group where X is —O— or —NH—, or a



group; and R<sup>5</sup> is a hydrogen atom, an alkyl group, an aryl group, or the group:



wherein A, m, R<sup>1</sup>, R<sup>2</sup>, R<sup>3</sup> and R<sup>4</sup> are as described above; or (2) a polymeric compound consisting essentially of recurring units with structures selected from:



wherein m, A, and R<sup>1</sup> and R<sup>4</sup> taken individually are as described above or R<sup>1</sup> and R<sup>4</sup> taken together with the carbon atoms to which they are attached form a



group; R<sup>6</sup> is an alkylene group; G is a carboxymethylmethylene group, a carboxyethylene group, or a group having the structure:



wherein m, A, and R<sup>1</sup> and R<sup>4</sup> taken individually are as described above; R<sup>7</sup> is an alkylene, cycloalkylene or arylene group which is the condensation residue of a diol or a diamine; and x is an integer of 1 or 2 and must be 1 only when G is the group:



wherein R<sup>1</sup> and R<sup>4</sup> are taken together with the carbon atoms to which they are attached to form a



group;

II



wherein  $m$ , A, and  $R^1$  and  $R^4$  taken individually are as described above;  $R^9$  is an alkylene group having 1 to 6 carbon atoms; Y is an —O— or —NH— group; and  $R^{10}$  is the condensation residue of a dicarboxylic acid;

III



wherein A, and  $R^1$  and  $R^4$  taken individually are as described above; and  $R^{12}$  is an alkylene group containing an ester or amido linkage; and

IV



wherein  $m$ , A, and  $R^1$  and  $R^4$  taken individually are as described above, and  $R^1$  and  $R^4$  when taken together with the carbon atoms to which they are attached are a



group;  $R^{13}$  is selected from any of the groups described for  $R^{12}$  and from groups having the structure:



wherein  $m$ , A,  $R^{12}$ , and  $R_1$  and  $R_4$  taken individually, are as described above, or when  $R^1$  and  $R^4$  are taken together with the atoms to which they are attached to form a



group,  $R^{13}$  is an alkylene, arylene, arylenebisalkylene, or an alkylenebisarylene group; and the sulfoxide and sulfone oxidation products of the above compounds.

2. The photographic silver halide emulsion of claim 1 containing the compound copoly[bicyclo[2.2.1]-5-heptene-2,3-dicarboxylic acid anhydride-bis(2-mercaptoethylsulfide-hexamethylene diamine].

3. The photographic silver halide emulsion of claim 1 containing the compound copoly[1,2-bis(2-mercaptoethoxy)ethanododecylhydro - 1,4:5,8 - dimethanoanthraquinonylene-2,6(or 7)].

4. The photographic silver halide emulsion of claim 1 containing the compound 5-carboxymethylmercapto-bicyclo[2.2.1]-heptene-2,3-dicarboximide.

5. The photographic silver halide emulsion of claim 1 containing the compound 5,5'(or 5,6')-sulfonylbis(bicyclo[2.2.1]heptane-2,3-dicarboxylic acid anhydride).

6. A photographic composition according to claim 1 wherein said compound is the polymeric condensation product of 1,8-bis(2,3-oxydicarbonylnorborn-5-ylthio)-3,6-dioxaoctane; 1-(1,2-oxydicarbonylethylthio)-8-(2,3-dicarboxynorborn-5-ylthio)-3,6-dioxaoctane; 1,8-bis(1,2-oxydicarbonylethylthio)-3,6-dioxaoctane; and 1,6-hexylenediamine.

7. A photographic composition according to claim 1 wherein said compound is the polymeric condensation product of 1,8-bis(2,3-oxydicarbonylnorborn-5-ylthio)-3,6-dioxaoctane and piperazine.

8. A photographic composition according to claim 1 wherein said compound is the polymeric condensation product of 1,8-bis(2,3-oxydicarbonyl-7-oxabicyclo[2.2.1]hept-5-ylthio)-3,6-dioxaoctane and 1,6-hexylenediamine.

9. A photographic composition according to claim 1 wherein said compound is 1,8-bis(2,3-dicarboxynorborn-5-ylthio)-3,6-dioxaoctane.

10. A photographic composition according to claim 1 wherein said compound is 2-carboxymethylthionorbornane.

11. A photographic composition according to claim 1 wherein said compound is 2,5(6)-dimercaptonorbornane.

12. A photographic composition according to claim 1 wherein said compound is 2,6(7)-dimercapto-1,4:5,8-dimethanoperhydronaphthalene.

13. A photographic composition according to claim 1 wherein said compound is 2-hydroxymethyl-5(6)-mercaptonorbornane.

14. A photographic composition according to claim 1 wherein said compound is poly[2-(1,2-dicarboxyethylthio)-5(6)-hydroxymethylthionorbornane].

15. A photographic composition according to claim 1 wherein said compound is poly[2-carboxy-3-methyl-5(6)-(2-hydroxymethyl-3-methylnorborn-5(6)-ylthio)norbornane].

16. A photographic composition according to claim 1 wherein said compound is poly[2,2-bis(hydroxymethyl)-3-methyl-5(6)-(1,2-dicarboxyethylthio)norbornane].

17. A photographic composition according to claim 1 wherein said compound is 5-acetylthionadic anhydride.

18. A photographic composition according to claim 1 wherein said compound is 2,5(6)-bis(acetylthio)norbornane.

19. A photographic composition according to claim 1 wherein said compound is 2,6(7)-bis(acetylthio)-1,4:5,8:9,10-trimethanoperhydroanthracene.

20. The photographic silver halide emulsion of claim 1 containing the compound copoly[bicyclo[2.2.1]-5-heptene-2,3-dicarboxylic anhydride-hexamethylene diamine-bis(2-mercaptoethoxy)ethane].

21. The photographic silver halide emulsion of claim 1 containing the compound copoly[bicyclo[2.2.1]-5-heptene-2,3-dicarboxylic anhydride-ethylene diamine-bis(2-mercaptoethoxy)ethane].

22. The photographic silver halide emulsion of claim 1 containing the compound copoly[bicyclo[2.2.1]-5-heptene-2,3-dicarboxylic anhydride-hexamethylene diamine-bis(1,2-mercapto)propanol].

23. The photographic silver halide emulsion of claim 1 containing the compound copoly[bicyclo[2.2.1]-5-hep-

27

tene-2,3-dicarboxylic anhydride-2-methyl - 2 - aminomethylbicyclo-5-heptene-bis(2-mercaptopethoxy)ethane].

24. The photographic silver halide emulsion of claim 1 containing the compound 2,6(or 7)di(carboxymethylmercapto)dodecahydro-1,4:5,8-dimethanoanthraquinone.

25. The photographic silver halide composition of claim 1 containing the polymeric compound having the formula:



10

wherein  $n$  is a positive integer.

26. The photographic silver halide composition of claim 1 containing the polymeric compound having the formula:



15

wherein  $n$  is a positive integer.

27. The photographic silver halide composition of claim 1 containing the polymeric compound having the formula:



wherein  $n$  is a positive integer.

28. The photographic silver halide emulsion of claim 1 containing the compound 5,5'-(or 5,6')-thiobis[bicyclo-[2.2.1]-5-heptane-2,3-dicarboxylic acid].

29. A silver halide photographic composition according to claim 1 wherein said compound is a polymeric compound having recurring units of the structure:



30

wherein  $m$  is an integer from 1 to 4, A is methylene group, an oxygen atom, a sulfur atom or an -NH group, R<sup>1</sup> and R<sup>4</sup> when taken individually are each a hydrogen atom, an alkyl, carboxy, mercapto, cyano, acylthio, or an alkanol group, or R<sup>1</sup> and R<sup>4</sup> taken together with the carbon atoms to which they are attached form a



35

group, R<sup>6</sup> is an alkylene group, G is a carboxymethylene group, a carboxyethylene group, or a group having the structure



28

where  $m$ , A, R<sup>1</sup> and R<sup>4</sup> taken individually are as described above, R<sup>7</sup> is an alkylene, cycloalkylene or arylene group which is the condensation residue of a diol or a diamine, and  $x$  is an integer of 1 or 2 and must be 1 only when G is the group:



45

wherein R<sup>1</sup> and R<sup>4</sup> are taken together with the carbon atoms to which they are attached to form a



50

group.

30. A photographic composition according to claim 29 wherein said compound is the polymeric condensation product of 1,8-bis(2,3 - oxydicarbonylnorborn-5-ylthio)-3-thiopentane and 1,6-hexylenediamine.

31. A photographic composition according to claim 29 wherein said compound is the polymeric condensation product of 1,8-bis(2,33-oxydicarbonylnorborn-5-ylthio)-3,6-dioxaoctane and 1,6-hexylenediamine.

32. A photographic composition according to claim 29 wherein said compound is the polymeric condensation product of 1,8-bis(2,33-oxydicarbonylnorborn-5-ylthio)-3,6-dioxaoctane and 1,2-ethylenediamine.

33. A photographic composition according to claim 29 wherein said compound is the polymeric condensation product of 1,2-bis(2,3-oxydicarbonylnorborn-5-ylthio)-2-hydroxymethylethane and 1,6-hexylenediamine.

34. A photographic composition according to claim 29 wherein said compound is the polymeric condensation product of 1,8-bis(2,3-oxydicarbonylnorborn-5-ylthio)-3,6-dioxaoctane and 1,8-bis(aminomethyl-2-methylnorborn-5(6)-ylthio)-3,6-dioxaoctane.

35. A photographic composition according to claim 29 wherein said compound is copoly[1,2-bis(2-mercaptopethoxy)ethanododecahydro - 1,4:5,8 - dimethanoanthraquinonylene-2,6(7)].

#### References Cited

##### UNITED STATES PATENTS

- |    |           |         |                       |          |
|----|-----------|---------|-----------------------|----------|
| 65 | 3,411,913 | 11/1968 | Faber et al. -----    | 96—109 X |
|    | 3,008,829 | 11/1961 | Clementi et al. ----- | 96—109 X |
|    | 3,043,697 | 7/1962  | Forsgard -----        | 96—109   |
|    | 3,544,327 | 12/1970 | Abel -----            | 96—109   |
|    | 3,459,549 | 8/1969  | McBride et al. -----  | 96—109 X |

70 NORMAN G. TORCHIN, Primary Examiner

W. H. LOUIE, Jr., Assistant Examiner

U.S. CL. X.R.

75 260—514, 268, 557, 455